

## UNITED STATES PATENT OFFICE

1,932,859

## ALUMINUM ALLOYS

Robert T. Wood, Cleveland, Ohio, assignor to  
Aluminum Company of America, Pittsburgh,  
Pa., a corporation of Pennsylvania

No Drawing. Original application September 21,  
1932, Serial No. 634,155. Divided and this ap-  
plication November 30, 1932. Serial No.  
645,113

2 Claims. (Cl. 75—1)

This invention relates to aluminum base al-  
loys containing magnesium. The invention has  
for its object the improvement of alloys of this  
class by the addition thereto of about 0.05 to 2.0  
5 per cent by weight of calcium. The invention  
is particularly concerned with the specific alloys  
hereinafter described.

The claims of this application cover certain  
matter divided from my copending application  
10 Serial No. 634,155 which is, in part, a continuation  
of my copending application Serial No. 595,-  
231. Inventions disclosed but not claimed here-  
in are claimed in my copending applications  
Serial Nos. 595,231, filed February 25, 1932, 645,-  
15 108 to 645,112 inclusive, and 645,114 to 645,125  
inclusive, all filed November 30, 1932.

Considerable difficulty has heretofore been en-  
countered in attempts to commercially produce  
castings of aluminum base alloys containing  
20 substantial amounts of magnesium. This diffi-  
culty is encountered both in the making of sand  
castings and permanent mold or chill-mold  
castings, although the nature of the difficulty  
differs somewhat in each case. In the case of  
25 sand castings there occurs a reaction between the  
molten aluminum base alloy containing mag-  
nesium and the ordinary sand-mold materials,  
or vapors generated therefrom. There is also a  
reaction with the atmosphere. In addition,  
30 the magnesium-containing aluminum base al-  
loy does not flow freely through narrow mold  
sections at ordinary pouring temperatures and,  
if the pouring temperature be raised, the solidified  
alloy is unsound. If the aluminum base  
35 alloy containing magnesium be cast in a chill-  
mold the reaction effect is minimized to some  
extent, but the troubles arising from cold-shuts  
and mis-runs are accentuated because of the  
more rapid chilling of the molten metal. The  
40 considerations apply to the aluminum base al-  
loys specifically disclosed herein and particu-  
larly to such alloys.

I have discovered that when calcium is added  
to aluminum base alloys of the type and com-  
45 position herein described, these difficulties are,  
to a considerable extent, eliminated. The cal-  
cium should be present in amounts ranging from  
0.05 per cent to 2.0 per cent by weight subject  
to specific considerations as hereinafter dis-  
50 closed.

In the melting of aluminum alloys of the com-  
positions herein described, a viscous scum often  
forms at the surface of the molten metal. Fail-  
ure of the molten metal to run properly through  
55 narrow mold apertures is caused, in part, by

shreds or particles of this scum being sus-  
pended in the molten metal and offering a re-  
sistance to the free passage of the metal through  
the apertures. Regardless of the cause of this  
low fluidity, I have discovered that the addi-  
tion to the alloy of relatively small amounts of  
calcium, in the preferred range between 0.05 to  
0.5 per cent, improves the casting characteristics  
to a very considerable extent and simultane-  
ously effects a reduction of the scum or dross col-  
lecting at or near the surface. In the casting  
of articles in sand molds, I prefer to add cal-  
cium in amounts less than about 0.5 per cent  
except, in instances where some reduction of  
tensile strength or other mechanical or tensile  
property is immaterial. In amounts of more  
than 0.5 per cent the calcium addition produces  
the advantages enumerated herein but has a  
tendency to lower some of the physical proper-  
ties of the alloys. This effect is not harmful  
when calcium is present in amounts of about  
0.5 per cent or less, but when high strength  
is not a desideratum the calcium may be used  
in amounts up to about 2.0 per cent. In intricate  
permanent mold castings, where casting  
troubles are very serious if no calcium be added,  
the improved physical properties obtained co-  
incident with the production of good castings  
more than offset the diminution in properties  
which might otherwise result from the use of  
the calcium.

I have also discovered that when calcium is  
added to aluminum base alloys containing mag-  
nesium, the amount of gas evolved during solidi-  
fication of the alloys is considerably reduced.  
When from about 0.05 per cent to 2.0 per cent  
by weight of calcium is added to the alloys, the  
amount of gas evolved becomes less marked  
with increasing calcium content and the reduc-  
tion of gas evolution may be so marked that the  
molten metal cools to the solidification tempera-  
ture with a smooth mirror-like surface. I pre-  
fer to restrict the amount of calcium added to  
2.0 per cent or less since above this amount  
the physical properties of the alloys may be too  
seriously affected. If the best physical prop-  
erties are desired with an improved, although  
not complete, degree of gas prevention, I keep  
the calcium content of the alloys between 0.05  
per cent and about 0.5 per cent.

In the application of the principles of my in-  
vention I have determined that certain  
aluminum base alloys containing magnesium are  
particularly benefited thereby. For example, a  
very useful aluminum base alloy is one con-

taining about 2.0 to 9.0 per cent of magnesium and 0.05 per cent to 2.0 per cent of calcium, as is also aluminum base alloy containing about 2.0 to 15.0 per cent of magnesium, 0.1 to 3.5 per cent of cobalt, and 0.05 to 2.0 per cent of calcium to which other elements such as copper, antimony, bismuth, nickel, manganese, and other well known alloying elements may be added to produce particular properties therein.

10 Likewise is the addition of 0.05 to 2.0 per cent of calcium beneficial to those aluminum base alloys which contain about 2.0 to 15.0 per cent of magnesium and 0.05 to 0.4 per cent of at least one of the class of metals here defined as 15 antimony and bismuth, such alloys being very useful where use at high temperatures is contemplated. Calcium may likewise be added to improve such alloys when they contain, in addition to magnesium and antimony and/or bis- 20 muth, one or more of such alloying elements as cobalt, copper, nickel, manganese, zinc, etc. which may be added to modify or produce a specific property in the alloy.

The addition of 0.05 to 2.0 per cent of calcium 25 is very beneficial in the case of a series of aluminum base alloys which contain as major alloying elements about 2.0 to 10.0 per cent of magnesium and about 0.2 to 5.0 per cent of nickel. For instance, an aluminum base alloy containing 30 3.0 to 7.5 per cent of magnesium and 0.2 to 2.0 per cent of nickel is improved by the addition of 0.05 to 2.0 per cent of calcium as is, likewise, this same alloy when it also contains about 0.05 to 0.4 per cent of one or more of the 35 class of elements composed of antimony and bismuth. Another excellent aluminum base alloy prepared in accordance with the principles of my invention is one containing 3.0 to 8.0 per cent of magnesium, 0.5 to 4.0 per cent of nickel, 40 0.5 to 4.0 per cent of manganese, and 0.05 to 2.0 per cent of calcium, which alloy may also be improved, particularly for application at high temperatures, by the addition of 0.05 to 0.4 per cent of at least one of the class of elements 45 composed of antimony and bismuth.

The principles of my invention find particular application in the case of aluminum base alloys containing magnesium, nickel, and chromium, and aluminum base alloys containing magnesium, nickel, and copper, as well as those alloys containing magnesium, nickel, and cobalt. Examples may be given of aluminum base alloys containing 2.0 to 10.0 per cent of magnesium, 0.2 to 5.0 per cent of nickel, 0.5 to 3.5 per cent of 50 chromium, and 0.05 to 2.0 per cent of calcium. An aluminum base alloy containing 3.0 to 8.0 per cent of magnesium, 0.5 to 3.5 per cent of nickel, 0.5 to 3.5 per cent of chromium, and 0.05 to 2.0 per cent of calcium has excellent casting properties 55 and the high temperature properties of this alloy can be favorably affected by the addition of 0.05 to 0.4 per cent of at least one of a class of elements composed of bismuth and antimony. Examples may be given of aluminum base alloy 60

65

containing 2.0 to 10.0 per cent of magnesium, 0.2 to 5.0 per cent of nickel, 1.0 to 6.0 per cent of copper, and 0.05 to 2.0 per cent of calcium. An excellent alloy of this type is one containing 3.0 to 8.0 per cent of magnesium, 0.5 to 5.0 per cent of nickel, 1.0 to 6.0 per cent of copper, and 0.05 to 2.0 per cent of calcium with or without 70 0.05 to 0.4 per cent of at least one of the class of elements composed of antimony and bismuth and with or without the further addition of 0.5 to 3.5 per cent of at least one of a class of elements composed of cobalt and chromium, and with or without the further addition of 0.1 to 1.0 per cent of at least one of a class of elements composed of tungsten, vanadium, molybdenum, titanium, and zirconium. 75

Other excellent alloys are those aluminum base alloys containing about 2.0 to 10.0 per cent magnesium, 0.2 to 5.0 per cent nickel, 0.1 to 3.5 per cent cobalt, and 0.05 to 2.0 per cent of calcium. A particular example of this class of alloys, which may also contain with considerable advantage 0.05 to 0.4 per cent of a class of elements composed of antimony and bismuth, is the aluminum base alloy containing 3.0 to 8.0 per cent magnesium, 0.5 to 4.0 per cent nickel, 0.1 to 3.0 per cent cobalt, and 0.05 to 2.0 per cent calcium. 90

Among other magnesium-containing aluminum base alloys which I have found to be particularly benefited by the presence of calcium are numbered the aluminum base alloys containing 3.0 to 8.0 per cent of magnesium, 1.0 to 6.0 per cent of copper, 0.5 to 3.5 per cent of chromium, and 0.05 to 2.0 per cent of calcium, with or 100 without the addition of 0.05 to 0.4 per cent of at least one of a class of metals composed of antimony and bismuth and with or without the addition of other alloying elements. 105

The alloys herein described may be produced 115 by the usual methods of alloying metals. The calcium is preferably added to the molten alloy by thrusting the calcium beneath the surface with tongs or other suitable instrument. The aluminum used in preparing the alloys may be 120 pure or it may contain the impurities found in commercial grades of this metal. Ordinarily a good commercial grade of virgin aluminum will give excellent results and is preferable. 125

Having thus explained and described my invention, I claim:

1. A metallic alloy consisting of 2.0 to 10.0 per cent by weight of magnesium, 0.2 to 5.0 per cent by weight of nickel, 0.5 to 3.5 per cent by weight of chromium, and 0.05 to 2.0 per cent by weight of calcium, the balance being aluminum. 130

2. A metallic alloy consisting of 3.0 to 8.0 per cent by weight of magnesium, 0.5 to 3.5 per cent by weight of nickel, 0.5 to 3.5 per cent by weight of chromium, and 0.05 to 2.0 per cent by weight of calcium, the balance being aluminum. 135

ROBERT T. WOOD.

140

70

145

75

150